

Patented July 10, 1928.

1,676,384

# UNITED STATES PATENT OFFICE.

HENRY THOMAS CHANDLER, OF NEW YORK, N. Y.

## BEARING STEEL.

No Drawing.

Application filed May 27, 1927. Serial No. 184,888.

This invention relates to the metallurgy of steel, and more particularly to a steel having new and improved mechanical characteristics, especially suitable for roller bearing rolls and races.

Steel which has been rolled or forged possesses directional properties, that is, the values of the physical properties of the steel will be different when measured in the direction of rolling, than when measured transversely to this direction.

The ultimate structural cause of this has its origin in the dendritic or other segregation occurring during solidification of the ingot. The solidification of molten steel proceeds differentially by the deposition about nuclei of solid layers increasing progressively in richness thereby producing local enrichments comprising concentrations of (1) non metallic impurities including slag, oxides, sulphides, etc.; (2) carbon, phosphorous, manganese, and the other elements of composition which occur in the ingot; (3) unwelded blowholes, and (4) defects such as seams, cracks and roll marks.

When the ingot is subsequently rolled or forged, these concentrations are drawn out in the direction of rolling or working, and there results a difference between the transverse and longitudinal chemical and physical characteristics of the bar, and consequently, a difference between its transverse and longitudinal physical structure and properties.

Any difference between the transverse and longitudinal properties of steel which has been hot worked, is metallurgically designated by the term "fiber" and it is this definition of the word which is understood in this description. The term "fiber" is used to describe this phenomenon inasmuch as the metal behaves as though composed of a system of fibers or stratifications because of the presence of elongated constituents, impurities or defects.

The fibrous structure of rolled steel persists, and in some cases is accentuated after heat treatment through a resulting additional concentration of carbides which, in the case of steels containing free cementite, is microscopically visible in the form of cementite-rich bands.

In general, the useful engineering properties of a bar of rolled steel are better when measured longitudinally, or in the direction of the rolling, than when measured

transversely thereto. Especially is this true in the case of the physical properties expressed by the terms, strength, impact value, fatigue resistance, and toughness. The magnitudes of these differences are determined by a number of variables which are known to those skilled in the art of applied metallurgy.

In the case of roller bearing rolls or races or ball bearing races made from rolled bar or tubing, in which the axis of rotation of the bearing is identical with, or substantially parallel to the direction of fiber in the bar, this longitudinal distribution of fiber operates adversely in the functioning of the part, due both to its influence on the surface properties of the bearing, and on the mechanical properties of the part considered as a whole.

With such bearings, many of the failures which result in use, as well as the limitations of service to which the bearing may be subjected, are determined by the nature and extent of the fiber in the steel.

Roller bearing rolls and their cooperating races, in service, are subjected to heavy dynamic stresses, impact and fatigue, which are exerted transversely to the axis of rotation.

The quality of such a bearing to resist destructive forces is, therefore, largely determined by the values of the transverse properties of the bar from which they are made. Not only are the values of the transverse properties, described by the terms, strength, impact value, fatigue resistance and toughness in general less than the values of the corresponding longitudinal properties, but due to the causes which produce this difference they are by nature more variable, and are to a lesser degree defined by chemical analysis and heat-treatment or the other qualifications generally used to specify a steel.

In the above mentioned bearings, the line of contact of the roller with its cooperating bearing surface, passes progressively over the various longitudinally extending fibers individually, substantially parallel thereto and consequently tends to pass over the individual fibers in sequence.

These fibers are not equally suitable to resist wear, and the other destructive forces acting upon the surface of the roller or the race, with the result that failure will start when the limit of endurance of the weakest

fiber functioning is reached, and rapidly to extend in the desired direction. It may in some instances be preferable to further work the member after twisting, either by forging or additional rolling. Hot twisting is generally preferable to cold, and may be advantageously done at some stage in the rolling process.

Many defects of rolled steel such as hair-line cracks, seams, and the like which extend longitudinally in the bar in the direction of rolling and are detrimental to the life and service of a roller bearing or race.

This is accomplished by causing the fibers to extend at an angle to the longitudinal axis of the roller, or of the race, or of both, whereby the line of contact instead of passing over each fiber separately, will act upon a plurality of adjacent fibers simultaneously.

13 The resistance to the destructive forces are thereby determined by the average resistance to the various fibers rather than by that of the weakest fiber.

Although the novel features which are believed to be characteristic of this invention will be particularly pointed out in the claim appended hereto, the invention itself, as to its objects and advantages, the mode of its operation and the manner of its organization 18 may be better understood by referring to the following description in which a particular commercial embodiment thereof is disclosed. It will be understood, however, that the processes and the steps thereof may be modified in various respects without departing from the broad spirit and scope of the invention.

In the following description and in the claim the various steps in the process and 23 the details comprising the invention will be identified by specific names for convenience, but they are intended to be as generic in their application as the art will permit.

One method of practicing this invention 28 comprises forming a steel rod by rolling or forging in the usual manner, so as to produce longitudinally extending fibers and subsequently further working the metal by mechanically twisting the completed bar 33 whereby the longitudinal fibers may be caused to extend helically around the axis thereof. After the steel bar has thus been treated, the roller or race is made therefrom by machining, heat-treating and grinding in the usual manner.

The physical and chemical structure of a bar thus treated consists of a mass of helically distributed fiber instead of the longitudinally distributed fiber of the usual rolled 38 bar.

The transverse axis of the bar thus treated therefore does not coincide with the transverse axis of the fibers themselves, and consequently the properties of such a bar in the 43 transverse direction are improved.

Obviously, various methods may be employed for imparting the above mentioned characteristics to a steel member, such as, for example producing the twist by the action 48 of the mill rolls in order to cause the fibers

in some applications of roller bearings, as for example, railroad car axles, a high degree of toughness and impact resistance is required to withstand the pounding action of the wheels on the rails, in addition to the high wear hardness necessary to reasonable service.

In such cases it is desirable to use a steel containing free carbides imbedded in a relatively tough matrix, the carbides, due to their hardness, supplying the necessary wear resistance, while the matrix is made sufficiently strong and tough to withstand the pounding action.

The use of such steel in the ordinary roller bearing has heretofore been expensive owing to the tendency of the free carbides to precipitate in bands parallel to the fiber, resulting in a surface alternately rich and poor in carbide concentration necessitating a comparatively large rejection. The line of contact between the roller and race consequently alternately passed over areas either deficient or too rich in carbides, and the wear was non-uniform and destruction was rapid.

In accordance with the present invention whereby the bands and fibers are caused to extend helically around the member, the line of contact extends at an angle to the carbide bands, and is at all times passing over a plurality of such bands whereby the carbide concentration along the line remains substantially constant. The fibers are arranged more advantageously with respect to the requirements of service, resulting in a bearing having a greater resistance to wear, impact, shock, and surface fatigue. In addition, steels having valuable characteristics which cannot at present be used in bearings of this type, due to their tendency to banding of carbides, are made available, and the effects of their line cracks, seams, slag threads and other metallurgical defects of rolled bars are rendered less harmful and the harmful effects of these defects are greatly lessened due to their helical distribution about the axis of rotation.

This invention may be applied to other structures than a steel rod, as for example, the races of a roller bearing. Such races are usually formed from a tubular member which has been heat-treated and rolled so as to produce a structure comprising longitudinally extending fibers as set forth above. According to my invention these fibers may be caused to extend helically around the surface of the roller by twisting the same, either cold or hot prior to cutting the vari-

ous races therefrom, or if made from a forging, after the part is formed. The line contact of the roller passing over the surface of a race will then cross a plurality of fibrous lines at an angle instead of crossing each fiber individually as heretofore.

Bearings constructed in accordance with this invention are of a more uniform quality inasmuch as many of the defects which may cause failures in the bearings are either eliminated or the effect thereof is minimized. Consequently, the degree of perfection required in the steel which is to be employed in bearings of this type is lower than that which would have been required for previous bearings and the percentage of useful metal obtained in a given mass is increased. Obviously if a bearing steel must be rigidly inspected for defects and must be discarded if any marked banding appears, the percentage of a given quantity of steel which could be employed for manufacture of bearings would be comparatively small. The present invention, however, distributes any segregated elements and redistributes the banding in such a manner that the detrimental effect thereof is reduced to a minimum. Thus a higher commercial yield may be obtained and the cost of production decreased accordingly.

A further advantageous feature of steel made in accordance with this invention resides in the fact that it is more resistant to shock or impacts and other stresses which are

applied in the transverse direction and since the stresses in the roller-bearings occur principally in that direction, the useful strength of the steel is materially increased. It is, therefore, possible to manufacture bearings which may be subjected to more severe service than was the case with bearings constructed from steel as heretofore employed. This is particularly true in railroad work where forces due to shock and impact are especially severe.

Although one process for making the improved product has been set forth and described and is pointed out in the claim, it is obvious that various changes may be made in the process or in the separate steps thereof without modifying or changing the essential features and characteristics of the product produced and that such product remains substantially the same although slight modifications may be made in its appearance, texture, and in its physical and chemical characteristics.

What is claimed is:

A roller bearing formed from a rod having free carbides in such proportion that said rod is unsuitable for bearing purposes, said rod being twisted whereby the lines of segregation of said carbides extend helically thereabout to produce a rod suitable for bearing purposes.

In testimony whereof I have hereunto set my hand.

HENRY THOMAS CHANDLER.